

## UNITED STATES PATENT OFFICE.

GEORGE I. RAY, OF CHARLOTTE, NORTH CAROLINA, ASSIGNEE TO RADIATOR SPECIALTY COMPANY, OF CHARLOTTE, NORTH CAROLINA, A CORPORATION OF NORTH CAROLINA.

## LEAK-STOPPING COMPOSITION.

No Drawing.

Application filed April 12, 1927. Serial No. 183,239.

This invention relates to a composition for stopping leaks in hot water circulating systems such as automobile radiators, cylinder blocks in internal combustion engines, 5 boilers, and in any other systems where hot water circulates.

Heretofore many leak stopping compositions have been manufactured and sold, but in many of these compositions the ingredients will settle in the lowest portion of the 10 hot water circulating system, clogging the same, and in many instances, the mucilaginous matter contained therein will form a coating over the interior of the circulating 15 system, which prevents radiation to a large extent and in the case of automobile radiators the radiators are so affected that it is sometimes necessary to clean the same before they can be used to any satisfaction.

20 It is an object of this invention to provide a composition for stopping leaks in hot water circulating systems which will permanently seal the leaks which may be present therein, and at the same time keep the 25 interior of the hot water circulating system in good condition.

Another object of my invention is to provide a leak stopping compound for hot water circulating systems which will repair 30 the leak without injury to the hot water circulating system.

Some of the objects of my invention having been stated, other objects will appear 35 when taken in connection with the accompanying description setting forth a preferred embodiment of my invention.

I attain the above stated objects of invention by placing in the hot water circulating system a composition which comprises the following ingredients:

|                                    | Per cent. |
|------------------------------------|-----------|
| Aluminum approximately             | 15        |
| Flax seed meal approximately       | 60        |
| Tri-sodium phosphate approximately | 20        |
| Silicate of soda approximately     | 5         |

Although I do not desire to be bound by the explanation as to how the above ingredients act and react when placed in a hot water circulating system, I offer the following explanation, as to what I think takes place.

When the composition is placed in a hot water circulating system, the tri-sodium phosphate and silicate of soda very soon 55 dissolve and hydrolyze, forming sodium hy-

droxide, and in addition, the silicate of soda produces colloidal hydrated silica. The flax is partially dissolved, the remainder of the flax remaining undissolved, and a portion of the flax seed meal, especially the mucilaginous portion goes into colloidal solution. In the course of time some soap is probably formed from the sodium hydroxide and the oil in the flax, and an additional amount of soap is formed from the resinous matter of the flax seed meal and the sodium hydroxide. The colloidal material from the soap, the silicate and the mucilage will tend to counteract the tendency of the flax seed meal to settle in the lowermost portions of the system to cause stoppage of the circulations. These colloids also act to keep the aluminum suspended.

In the leak stopping process the larger portions of the flax seed meal find their way into the leaks and become lodged therein, the smaller particles follow the larger ones, and soon the hole is plugged. In the course of a very short time the sodium hydroxide acts on the aluminum, causing the latter to form aluminum hydroxide, aluminum soap, and aluminum silicate. All of these compounds aid in cementing the uncombined aluminum and flax seed particles in position, thus making the seals permanent.

I find that the deterging and cleansing action of both tri-sodium phosphate and silicate of soda is good, that of the silicate of soda, being especially good, since it produces the colloidal hydrated silica, as above mentioned.

In the specification, I have set forth a preferred embodiment of my invention, and although specific terms are employed, they are used in a generic and descriptive sense only, and not for purposes of limitation, the scope of the invention being set forth in the appended claims.

I claim:

1. A composition for stopping leaks in hot water circulating systems comprising a mixture of aluminum, flax seed meal, tri-sodium phosphate and silicate of soda.

2. A composition for stopping leaks in hot water circulating systems comprising a mixture of aluminum, flax seed meal and tri-sodium phosphate.

In testimony whereof I affix my signature.

GEORGE I. RAY.